# EUROPEAN PATENT SPECIFICATION

(11) **EP 2 503 571 B1**
(45) Date of publication and mention of the grant of the patent: **06.05.2015**
(21) Application number: 11765493.9
(22) Date of filing: 28.03.2011
(51) Int. Cl.: H01F 41/02, H01F 1/053, H01F 1/08, H01F 7/02, H02K 15/03

(54) **MANUFACTURING METHOD FOR PERMANENT MAGNET**
VERFAHREN ZUR HERSTELLUNG EINES PERMANENTMAGNETEN
PROCÉDÉ DE FABRICATION d'AIMANT PERMANENT

(30) Priority: 31.03.2010 JP 2010084094
(43) Date of publication of application: 26.09.2012
(73) Proprietor: Nitto Denko Corporation, Ibaraki-shi, Osaka 567-8680 (JP)
(72) Inventor: OZEKI Izumi, Ibaraki-shi Osaka 567-8680 (JP); KUME Katsuya, Ibaraki-shi Osaka 567-8680 (JP); HIRANO Keisuke, Ibaraki-shi Osaka 567-8680 (JP); OMURE Tomohiro, Ibaraki-shi Osaka 567-8680 (JP); TAIHAKU Keisuke, Ibaraki-shi Osaka 567-8680 (JP); OZAKI Takashi, Ibaraki-shi Osaka 567-8680 (JP)
(74) Representative: Grünecker Patent- und Rechtsanwälte PartG mbB
(86) International application number: PCT/JP2011/057574
(87) International publication number: WO 2011/125593

(56) References cited:
- WO-A1-2009/150843
- JP-A- 10 064 746
- JP-A- 10 214 711
- JP-A- 2004 281 873
- JP-A- 2006 270 087
- JP-A- 2009 032 742

## Description

### TECHNICAL FIELD

The present invention relates to a permanent magnet and manufacturing method thereof.

### BACKGROUND ART

In recent years, a decrease in size and weight, an increase in power output and an increase in efficiency have been required in a permanent magnet motor used in a hybrid car, a hard disk drive, or the like. To realize such a decrease in size and weight, an increase in power output and an increase in efficiency in the permanent magnet motor mentioned above, a further improvement in magnetic performance is required of a permanent magnet to be buried in the permanent magnet motor. Meanwhile, as permanent magnet, there have been known ferrite magnets, Sm-Co-based magnets, Nd-Fe-B-based magnets, Sm₂Fe₁₇Nₓ-based magnets or the like. As permanent magnet for permanent magnet motor, there are typically used Nd-Fe-B-based magnets among them due to remarkably high residual magnetic flux density.

As method for manufacturing a permanent magnet, a powder sintering process is generally used. In this powder sintering process, raw material is coarsely milled first and furthermore, is finely milled into magnet powder by a jet mill (dry-milling method) or a wet bead mill (wet-milling method). Thereafter, the magnet powder is put in a mold and pressed to form in a desired shape with magnetic field applied from outside. Then, the magnet powder formed and solidified in the desired shape is sintered at a predetermined temperature (for instance, at a temperature between 800 and 1150 degrees Celsius for the case of Nd-Fe-B-based magnet) for completion.

### PRIOR ART DOCUMENT

### PATENT DOCUMENT

Patent document 1: Japanese Registered Patent Publication No. 3298219 (pages 4 and 5)
Patent document 2: JP 2009 032742 A discloses the wet pulverization in isoparaffin of a high Dy-containing R-T-B alloy followed by degreasing at 150 °C in vacuum, later compacted and sintered.

### DISCLOSURE OF THE INVENTION

### PROBLEM TO BE SOLVED BY THE INVENTION

Meanwhile, it has been known that the magnetic performance of a permanent magnet can be basically improved by making the crystal grain size in a sintered body very fine, because the magnetic characteristics of a magnet can be approximated by a theory of single-domain particles. Here, in order to make the grain size in the sintered body very fine, a particle size of the magnet raw material before sintering also needs to be made very fine.

Here, the milling methods to be employed at the milling of the magnet raw material include wet bead milling, in which a container is rotated with beads (media) put therein, and slurry of the raw material mixed in a solvent is added into the container, so that the raw material is ground and milled. The wet bead milling allows the magnet raw material to be milled into a range of fine particle size (for instance, 0.1 µm through 5.0 µm).

However, in a wet milling method like the above wet bead milling, an organic solvent such as toluene, cyclohexane, ethyl acetate and methanol may be used as a solvent to be mixed with the magnet raw material. Accordingly, even if the organic solvent is volatilized through vacuum desiccation or the like after milling, carbon-containing material may remain in the magnet. Then, reactivity of neodymium (Nd) and carbon is significantly high and carbide is formed in case carbon-containing material remains even at a high-temperature stage in a sintering process. Consequently, there has been such a problem as thus formed carbide causes a gap between a main phase and a grain boundary phase, so that the entirety of the magnet cannot be sintered densely, drastically degrading magnetic performance thereof. Even if no gap is formed, there still be a problem that the formed carbide causes alpha iron to separate out in a main phase of a sintered magnet and magnetic properties are considerably degraded.

The invention has been made in order to solve the above-mentioned conventional problems, and an object of the invention is to provide a permanent magnet in which the magnet powder mixed with the organic solvent at the wet milling is calcined in a hydrogen atmosphere before sintering so that the amount of carbon contained in a magnet particle can be reduced in advance, enabling the entirety of the magnet to be densely sintered without making a gap between a main phase and a grain boundary phase in the sintered magnet.

### MEANS FOR SOLVING THE PROBLEM

In the above-described permanent magnet of the present invention, residual carbon content after sintering is 0.1 wt% or less.

To achieve the above object, the present invention provides in claim 1 a manufacturing method of a permanent magnet comprising steps of wet-milling magnet material in an organic solvent to obtain magnet powder; calcining the magnet powder in hydrogen atmosphere so as to obtain a calcined body; compacting the calcined body so as to form a compact body; and sintering the compact body.

In the above-described manufacturing method of a permanent magnet of the present invention, residual carbon content after sintering is 0.1 wt% or less.

### EFFECT OF THE INVENTION

According to the manufacturing method of a permanent magnet of the present invention, magnet powder mixed with organic solvent at the wet milling is calcined in a hydrogen atmosphere before sintering, so that the amount of carbon contained in a magnet particle can be reduced in advance. Consequently, the entirety of the magnet can be sintered densely without making a gap between a main phase and a grain boundary phase in the sintered magnet, and decline of coercive force can be avoided. Further, considerable amount of alpha iron does not separate out in the main phase of the sintered magnet and serious deterioration of magnetic properties can be avoided.

According to the manufacturing method of a permanent magnet of the present invention, the carbon content in the magnet powder can be reduced in advance as the magnet powder mixed with organic solvent at the wet milling in the manufacturing processes of the permanent magnet is calcined in hydrogen atmosphere before sintering. Consequently, the entirety of the magnet can be sintered densely without making a gap between a main phase and a grain boundary phase in the sintered magnet, and decline of coercive force can be avoided. Further, considerable amount of alpha iron does not separate out in the main phase of the sintered magnet and serious deterioration of magnetic properties can be avoided.

Further, since powdery magnet particles are calcined, thermal decomposition of the organometallic compound contained can be caused more easily in the entirety of the magnet particles in comparison with the case of calcining compacted magnet particles. In other words, carbon content in the calcined body can be reduced more reliably.

### BRIEF DESCRIPTION OF THE DRAWINGS

[FIG. 1] is an overall view of a permanent magnet of the disclosure.
[FIG. 2] is an enlarged schematic view in vicinity of grain boundaries of the permanent magnet of the disclosure.
[FIG. 3] is an explanatory diagram illustrating manufacturing processes of a permanent magnet according to a manufacturing method of the disclosure.
[FIG. 4] is an explanatory diagram illustrating manufacturing processes of a permanent magnet according to a manufacturing method of the invention.
[FIG. 5] is a diagram illustrating changes of oxygen content with and without a calcination process in hydrogen.
[FIG. 6] is a table illustrating residual carbon content in permanent magnets obtained by the manufacturing method of an embodiment and a comparative example.
[FIG. 7] is an SEM image and an element analysis result on a main phase and a grain boundary phase of the permanent magnet obtained by the manufacturing method of the embodiment after sintering.
[FIG. 8] is an SEM image and an element analysis result on a main phase and a grain boundary phase of the permanent magnet of the comparative example after sintering.

### BEST MODE FOR CARRYING OUT THE INVENTION

Specific embodiments of a method for manufacturing the permanent magnet according to the present invention will be described below in detail with reference to the drawings.

### [Constitution of Permanent Magnet]

First, a constitution of a permanent magnet 1 will be described. FIG. 1 is an overall view of the permanent magnet 1. Incidentally, the permanent magnet 1 depicted in FIG. 1 is formed into a cylindrical shape. However, the shape of the permanent magnet 1 may be changed in accordance with the shape of a cavity used for compaction.

As the permanent magnet 1, an Nd-Fe-B-based magnet may be used, for example. Further, as illustrated in FIG. 2, the permanent magnet 1 is an alloy in which a main phase 11 and an Nd-rich phase 12 coexist. The main phase 11 is a magnetic phase which contributes to the magnetization and the Nd-rich phase 12 is a low-melting-point and non-magnetic phase where rare earth elements are concentrated. FIG. 2 is an enlarged view of Nd magnet particles composing the permanent magnet 1.

Here, in the main phase 11, Nd₂Fe₁₄B intermetallic compound phase (Fe here may be partially replaced with Co), which is of a stoichiometric composition, accounts for high proportion in volume. Meanwhile, the Nd-rich phase 12 consists of an intermetallic compound phase having higher composition ratio of Nd than that of Nd₂Fe₁₄B (Fe here may be partially replaced with Co) of a stoichiometric composition, too (for example, Nd_{2.0-3.0}Fe₁₄B intermetallic compound phase) . Further, the Nd-rich phase 12 may include a small amount of other elements such as Dy, Tb, Co, Cu, Al, or Si for improving magnetic property.

Then, in the permanent magnet 1, the Nd-rich phase 12 has the following features. The Nd-rich phase 12:
(1) has a low melting point (approx. 600 degrees Celsius) and turns into a liquid phase at sintering, contributing to densification of the magnet, which means improvement in magnetization;
(2) can eliminate surface irregularity of grain boundaries, decreasing nucleation sites of reverse magnetic domain and enhancing coercive force; and
(3) can magnetically insulate the main phase, increasing the coercive force.

Poorly dispersed Nd-rich phase 12 in the sintered permanent magnet 1 potentially causes a partial sintering defect and degrade in the magnetic property; therefore it is important to have the Nd-rich phase 12 uniformly dispersed in the sintered permanent magnet 1.

An example of problems likely to rise when manufacturing the Nd-Fe-B-based magnet is formation of alpha iron in a sintered alloy. This may be caused as follows: when a permanent magnet is manufactured using a magnet raw material alloy whose contents are based on the stoichiometric composition, rare earth elements therein combine with oxygen during the manufacturing process so that the amount of rare earth elements becomes insufficient in comparison with the stoichiometric composition. Here, the alpha iron has a deformability and remains in a milling device without being milled, and accordingly, the alpha iron not only deteriorates the efficiency in milling the alloy, but also adversely affects the grain size distribution and composition variation before and after milling. Further, if alpha iron remains in the magnet after sintering, the magnetic property of the magnet is degraded.

It is thus desirable that the amount of all rare earth elements contained in the permanent magnet 1, including Nd, is within a range of 0.1 wt% through 10.0 wt% larger, or more preferably, 0.1 wt% through 5.0 wt% larger than the amount based upon the stoichiometric composition (26.7 wt%). Specifically, the contents of constituent elements are set to be Nd: 26.7 through 37 wt%, B: 1 through 2 wt%, Fe (electrolytic iron) : 60 through 75 wt%, respectively. By setting the contents of rare earth elements in the permanent magnet within the above range, it becomes possible to obtain the sintered permanent magnet 1 in which the Nd-rich phase 12 is uniformly dispersed. Further, even if the rare earth elements are combined with oxygen during the manufacturing process, the formation of alpha iron in the sintered permanent magnet 1 can be prevented, without shortage of the rare earth elements in comparison with the stoichiometric composition.

Incidentally, if the amount of rare earth elements contained in the permanent magnet 1 is smaller than the above-described range, the Nd-rich phase 12 becomes difficult to be formed. Also, the formation of alpha iron cannot sufficiently be inhibited. Meanwhile, in a case the content of rare earth elements in the permanent magnet 1 is larger than the above-described range, the increase of the coercive force becomes slow and also the residual magnetic flux density is reduced. Therefore such a case is impracticable.

Furthermore, in the present invention, so-called wet milling is performed in which magnet raw material put into the organic solvent is milled in the organic solvent, when the magnet material is milled into magnet powder of a very fine particle size. However, if the magnet material is milled wet in the organic solvent, even if the organic solvent is volatilized through vacuum desiccation performed later, an organic compound such as the organic solvent still remains in the magnet. In addition, reactivity of Nd and carbon is significantly high and in case carbon-containing material remains even at a high-temperature stage in a sintering process, carbide is formed. As a result, there is a problem that gaps are formed between the main phase and the grain boundary phase (Nd-rich phase) of the magnet after sintering due to the created carbide, making it impossible to densely sinter the entirety of the magnet, and thus significantly deteriorating the magnetic properties thereof. However, in the present invention, the carbon content in magnet particles can be reduced in advance through performing a later-described calcination process in hydrogen before sintering.

Further, it is desirable to set the crystal grain diameter of the main phase 11 to be 0.1 µm through 5.0 µm. Incidentally, the structure of the main phase 11 and the Nd-rich phase 12 can be confirmed, for instance, through scanning electron microscopy (SEM), transmission electron microscopy (TEM) or three-dimensional atom probe technique.

If Dy or Tb is included in the Nd-rich phase, coercive force can be improved by Dy or Tb inhibiting the reverse magnetic domain from forming in the grain boundaries.

### [First Method for Manufacturing Permanent Magnet]

Next, a method for manufacturing the permanent magnet 1 directed to the disclosure will be described below with reference to FIG. 3. FIG. 3 is an explanatory view illustrating a manufacturing process in a method for manufacturing the permanent magnet 1 directed to the disclosure.

First, there is manufactured an ingot comprising Nd-Fe-B of certain fractions (for instance, Nd: 32.7 wt%, Fe (electrolytic iron) : 65.96 wt%, and B: 1.34 wt%). Thereafter the ingot is coarsely milled using a stamp mill, a crusher, etc. to a size of approximately 200 µm. Otherwise, the ingot is dissolved, formed into flakes using a strip-casting method, and then coarsely milled using a hydrogen pulverization method. Thus, coarsely-milled magnet powder 31 is obtained.

Then, the coarsely milled magnet powder 31 is finely milled to a predetermined size (for instance, 0.1 µm -5.0 µm) by a wet method using a bead mill, and the magnet powder is dispersed in a solvent to prepare slurry 42. Incidentally, in the wet milling, 4 kg of toluene is used as a solvent to 0.5 kg of the magnet powder.

Incidentally, detailed dispersion conditions are as below.
Dispersing device: bead mill;
Dispersing media: zirconia beads.

Furthermore, the solvent used for milling is an organic solvent. However, there is no particular limitation on the types of solvent, and there can be used an alcohol such as isopropyl alcohol, ethanol or methanol, an ester such as ethyl acetate, a lower hydrocarbon such as pentane or hexane, an aromatic compound such as benzene, toluene or xylene, a ketone, a mixture thereof or the like.

Thereafter, the prepared slurry 42 is desiccated in advance through vacuum desiccation or the like before compaction and desiccated magnet powder 43 is obtained. Then, the desiccated magnet powder is subjected to powder-compaction to form a given shape using a compaction device 50. There are dry and wet methods for the powder compaction, and the dry method includes filling a cavity with the desiccated fine powder and the wet method includes filling a cavity with the slurry 42 without desiccation. In this embodiment, a case where the dry method is used is described as an example. Furthermore, the organic solvent can be volatilized at the sintering stage after compaction.

As illustrated in FIG. 3, the compaction device 50 has a cylindrical mold 51, a lower punch 52 and an upper punch 53, and a space surrounded therewith forms a cavity 54. The lower punch 52 slides upward/downward with respect to the mold 51, and the upper punch 53 slides upward/downward with respect to the mold 51, in a similar manner.

In the compaction device 50, a pair of magnetic field generating coils 55 and 56 is disposed in the upper and lower positions of the cavity 54 so as to apply magnetic flux to the magnet powder 43 filling the cavity 54. The magnetic field to be applied may be, for instance, 1 MA/m.

When performing the powder compaction, firstly, the cavity 54 is filled with the desiccated magnet powder 43. Thereafter, the lower punch 52 and the upper punch 53 are activated to apply pressure against the magnet powder 43 filling the cavity 54 in a pressurizing direction of arrow 61, thereby performing compaction thereof. Furthermore, simultaneously with the pressurization, pulsed magnetic field is applied to the magnet powder 43 filling the cavity 54, using the magnetic field generating coils 55 and 56, in a direction of arrow 62 which is parallel with the pressuring direction. As a result, the magnetic field is oriented in a desired direction. Incidentally, it is necessary to determine the direction in which the magnetic field is oriented while taking into consideration the magnetic field orientation required for the permanent magnet 1 formed from the magnet powder 43.

Furthermore, in a case where the wet method is used, slurry may be injected while applying the magnetic field to the cavity 54, and in the course of the injection or after termination of the injection, a magnetic field stronger than the initial magnetic field may be applied to perform the wet molding. Furthermore, the magnetic field generating coils 55 and 56 may be disposed so that the application direction of the magnetic field is perpendicular to the pressuring direction.

Secondly, the compact body 71 formed through the powder compaction is held for several hours (for instance, five hours) in hydrogen atmosphere at 200 through 900 degrees Celsius, or more preferably 400 through 900 degrees Celsius (for instance, 600 degrees Celsius), to perform a calcination process in hydrogen. The hydrogen feed rate during the calcination is 5 L/min. So-called decarbonization is performed during this calcination process in hydrogen. In the decarbonization, the remaining organic compound is thermally decomposed so that carbon content in the calcined body can be decreased. Furthermore, calcination process in hydrogen is to be performed under a condition of less than 0.1 wt% carbon content in the calcined body, or more preferably less than 0.05 wt%. Accordingly, it becomes possible to densely sinter the permanent magnet 1 in its entirety in the following sintering process, and the decrease in the residual magnetic flux density and coercive force can be prevented.

Here, NdH₃ exists in the compact body 71 calcined through the calcination process in hydrogen as above described, which indicates a problematic tendency to combine with oxygen. However, in the first manufacturing method, the compact body 71 after the calcination is brought to the later-described sintering without being exposed to the external air, eliminating the need for the dehydrogenation process. The hydrogen contained in the compact body is removed while being sintered.

Following the above, there is performed a sintering process for sintering the compact body 71 calcined through the calcination process in hydrogen. However, for a sintering method for the compact body 71, there can be employed, besides commonly-used vacuum sintering, pressure sintering in which the compact body 71 is sintered in a pressured state. For instance, when the sintering is performed in the vacuum sintering, the temperature is risen to approximately 800 through 1080 degrees Celsius in a given rate of temperature increase and held for approximately two hours. During this period, the vacuum sintering is performed, and the degree of vacuum is preferably equal to or smaller than 10⁻⁴ Torr. The compact body 71 is then cooled down, and again undergoes a heat treatment in 600 through 1000 degrees Celsius for two hours. As a result of the sintering, the permanent magnet 1 is manufactured.

Meanwhile, the pressure sintering includes, for instance, hot pressing, hot isostatic pressing (HIP), high pressure synthesis, gas pressure sintering, and spark plasma sintering (SPS) and the like. However, it is preferable to adopt the spark plasma sintering which is uniaxial pressure sintering in which pressure is uniaxially applied and also in which sintering is performed by electric current sintering, so as to prevent grain growth of the magnet particles during the sintering and also to prevent warpage formed in the sintered magnets. Incidentally, the following are the preferable conditions when the sintering is performed in the SPS; pressure is applied at 30 MPa, the temperature is risen in a rate of 10 degrees Celsius per minute until reaching 940 degrees Celsius in vacuum atmosphere of several Pa or lower and then the state of 940 degrees Celsius in vacuum atmosphere is held for approximately five minutes. The compact body 71 is then cooled down, and again undergoes a heat treatment in 600 through 1000 degrees Celsius for two hours. As a result of the sintering, the permanent magnet 1 is manufactured.

### [Inventive Second Method for Manufacturing Permanent Magnet]

Next, the method for manufacturing the permanent magnet 1 will be described below with reference to FIG. 4. FIG. 4 is an explanatory view illustrating a manufacturing process in the method for manufacturing the permanent magnet 1 directed to the present invention.

The process until the slurry 42 is manufactured is the same as the manufacturing process in the first manufacturing method already discussed referring to FIG. 3, therefore detailed explanation thereof is omitted.

Firstly, the prepared slurry 42 is desiccated in advance through vacuum desiccation or the like before compaction and desiccated magnet powder 43 is obtained. Then, the desiccated magnet powder 43 is held for several hours (for instance, five hours) in hydrogen atmosphere at 200 through 900 degrees Celsius, or more preferably 400 through 900 degrees Celsius (for instance, 600 degrees Celsius), for a calcination process in hydrogen. The hydrogen feed rate during the calcination is 5 L/min. So-called decarbonization is performed in this calcination process in hydrogen. In the decarbonization, the organometallic material is thermally decomposed so that carbon content in the calcined body can be decreased. Furthermore, calcination process in hydrogen is to be performed under a condition of less than 0.1 wt% carbon content in the calcined body, or more preferably less than 0. 05 wt%. Accordingly, it becomes possible to densely sinter the permanent magnet 1 in its entirety in the following sintering process, and the decrease in the residual magnetic flux density and coercive force can be prevented.

Secondly, the powdery calcined body 82 calcined through the calcination process in hydrogen is held for one through three hours in vacuum atmosphere at 200 through 600 degrees Celsius, or more preferably 400 through 600 degrees Celsius for a dehydrogenation process. Incidentally, the degree of vacuum is preferably equal to or smaller than 0.1 Torr.

Here, NdH₃ exists in the calcined body 82 calcined through the calcination process in hydrogen as above described, which indicates a problematic tendency to combine with oxygen.

FIG. 5 is a diagram depicting oxygen content of magnet powder with respect to exposure duration, when Nd magnet powder with a calcination process in hydrogen and Nd magnet powder without a calcination process in hydrogen are exposed to each of the atmosphere with oxygen concentration of 7 ppm and the atmosphere with oxygen concentration of 66 ppm. As illustrated in FIG. 5, when the Nd magnet powder with the calcination process in hydrogen is exposed to the atmosphere with high-oxygen concentration of 66 ppm, the oxygen content of the magnet powder increases from 0.4 % to 0.8 % in approximately 1000 sec. Even when the Nd magnet powder with the calcination process is exposed to the atmosphere with low-oxygen concentration of 7 ppm, the oxygen content of the magnet powder still increases from 0.4 % to the similar amount 0.8 %, in approximately 5000 sec. Oxygen combined with Nd causes the decrease in the residual magnetic flux density and in the coercive force.

Therefore, in the above dehydrogenation process, NdH₃ (having high activity level) in the calcined body 82 created at the calcination process in hydrogen is gradually changed: from NdH₃ (having high activity level) to NdH₂ (having low activity level). As a result, the activity level is decreased with respect to the calcined body 82 activated by the calcination process in hydrogen. Accordingly, if the calcined body 82 calcined at the calcination process in hydrogen is later moved into the external air, Nd therein is prevented from combining with oxygen, and the decrease in the residual magnetic flux density and coercive force can also be prevented.

Then, the powdery calcined body 82 after the dehydrogenation process undergoes the powder compaction to be compressed into a given shape using the compaction device 50. Details are omitted with respect to the compaction device 50 because the manufacturing process here is similar to that of the first manufacturing method already described referring to FIG. 3.

Then, there is performed a sintering process for sintering the compacted-state calcined body 82. The sintering process is performed by the vacuum sintering or the pressure sintering similar to the above first manufacturing method. Details of the sintering condition are omitted because the manufacturing process here is similar to that of the first manufacturing method already described. As a result of the sintering, the permanent magnet 1 is manufactured.

However, the second manufacturing method discussed above has an advantage that the calcination process in hydrogen is performed to the powdery magnet particles, therefore the thermal decomposition of the remaining organic compound can be more easily caused to the entire magnet particles, in comparison with the first manufacturing method in which the calcination process in hydrogen is performed to the compacted magnet particles. That is, it becomes possible to securely decrease the carbon content of the calcined body, in comparison with the first manufacturing method.

However, in the first manufacturing method, the compact body 71 after calcined in hydrogen is brought to the sintering without being exposed to the external air, eliminating the need for the dehydrogenation process. Accordingly, the manufacturing process can be simplified in comparison with the second manufacturing method.

### EMBODIMENTS

Here will be described an embodiment according to the present invention referring to a comparative example for comparison.

### (Embodiment)

In comparison with fraction regarding alloy composition of a neodymium magnet according to the stoichiometric composition (Nd: 26.7 wt%, Fe (electrolytic iron) : 72.3 wt%, B: 1.0 wt%), proportion of Nd in that of the neodymium magnet powder for the embodiment is set higher, such as Nd/ Fe/ B= 32.7/ 65.96/ 1.34 in wt%, for instance. Further, toluene is used as organic solvent for wet milling. A calcination process has been performed by holding the magnet powder before compaction for five hours in hydrogen atmosphere at 600 degrees Celsius. The hydrogen feed rate during the calcination is 5 L/min. Sintering of the compacted-state calcined body has been performed in the SPS. Other processes are the same as the processes in [Second Method for Manufacturing Permanent Magnet] mentioned above.

### (Comparative Example)

Toluene is used as organic solvent for wet milling. The magnet powder after wet-milling is compacted without the calcination process in hydrogen. Sintering of the compacted-state magnet powder has been performed in the SPS. Other conditions are the same as the conditions in embodiment.

### (Comparison of Embodiment with Comparative Example Regarding Residual Carbon Content)

The table of FIG. 6 shows residual carbon content [wt%] in each permanent magnet according to the embodiment and the comparative example.

As shown in FIG. 6, the carbon content remaining in the magnet particles can be significantly reduced in the embodiment in comparison with the comparative example. Specifically, the carbon content remaining in the magnet particles can be made 0.05 wt% or less in the embodiment.

Further, in comparison between the embodiment and the comparative example, despite the same organic compound is used for performing wet-milling, there are significant differences with respect to carbon content in magnet particles depending on with or without calcination process in hydrogen; the case with the calcination process in hydrogen can reduce carbon content more significantly than the case without. In other words, through the calcination process in hydrogen, there can be performed so-called decarbonization in which the organic compound is thermally decomposed so that carbon content in the calcined body can be decreased. As a result, it becomes possible to densely sinter the entirety of the magnet and to prevent the coercive force from degradation.

### (Result of Surface Analysis with XMA Carried Out for Permanent Magnets)

Surface analysis with an XMA (X-ray micro analyzer) has been carried out for each of permanent magnets directed to the embodiment and the comparative example. FIG. 7 is an SEM image and an element analysis result on a grain boundary phase of the permanent magnet of the embodiment after sintering. FIG. 8 is an SEM image and an element analysis result on a grain boundary phase of the permanent magnet of the comparative example after sintering.

Comparison will be made with the SEM images of the embodiment and the comparative example. With respect to the embodiment in which residual carbon content is equal to specific amount or lower (e.g., 0.1 wt% or less), there can be observed formation of a sintered permanent magnet basically constituted by a main phase of neodymium magnet (Nd₂Fe₁₄B) 91 and a grain boundary phase 92 that looks like white speckles. Also, a small amount of alpha iron phase is formed there. On the other hand, with respect to the comparative example in which residual carbon content is larger in comparison with the embodiment, there can be observed formation of considerable number of alpha iron phases 93 that look like black belts in addition to a main phase 91 and a grain boundary phase 92. It is to be noted that alpha iron is generated due to carbide that remains at the time of sintering. That is, reactivity of Nd and carbon is significantly high and in case carbon-containing material remains in the organic compound even at a high-temperature stage in a sintering process like the comparative example, carbide is formed. Consequently, the thus formed carbide causes alpha iron to separate out in a main phase of a sintered magnet and magnetic properties are considerably degraded.

On the other hand, as described in the above, the embodiment performs the calcination process in hydrogen so that the organic compound is thermally decomposed and carbon contained therein can be burned off previously (i.e., carbon content can be reduced). Especially, by setting calcination temperature to a range between 200 and 900 degrees Celsius, more preferably to a range between 400 and 900 degrees Celsius, carbon contained therein can be burned off more than required and carbon content remaining in the magnet after sintering can be restricted to the extent of less than 0.1 wt%, more preferably, less than 0.05 wt%. In the embodiment where carbon content remaining in the magnet is less than 0.1 wt%, little carbide is formed in a sintering process, which avoids the problem such like the appearance of the considerable number of alpha iron phases 93 that can be observed in the comparative example. Consequently, as shown in FIG. 7, the entirety of the permanent magnet 1 can be sintered densely through the sintering process. Further, considerable amount of alpha iron does not separate out in a main phase of the sintered magnet so that serious degradation of magnetic properties can be avoided.

Incidentally, if a permanent magnet is manufactured through wet-bead-milling without adding alkoxide, and sintering without hydrogen calcination, the remnant carbon in the permanent magnet is measured at 12000 ppm in a case toluene is used as solvent, and 31000 ppm in a case cyclohexane is used. Meanwhile, with hydrogen calcination, the remnant carbon can be reduced to approximately 300 ppm in either case of toluene or cyclohexane.

In the above embodiment and the comparative example, permanent magnets manufactured in accordance with [Second Method for Manufacturing Permanent Magnet] have been used. Similar results can be obtained in case of using permanent magnets manufactured in accordance with [First Method for Manufacturing Permanent Magnet].

As described in the above, with respect to the permanent magnet 1 and the manufacturing method of the permanent magnet 1 directed to the above embodiment, coarsely-milled magnet powder is further milled in a solvent by a bead mill. Thereafter, a compact body formed through powder compaction of the magnet powder is held for several hours in hydrogen atmosphere at 200 through 900 degrees Celsius for a calcination process in hydrogen. Thereafter, through sintering at 800 through 1180 degrees Celsius, the permanent magnet 1 is manufactured. Accordingly, even if an organic solvent is used in wet-milling of the magnet material, the remaining organic compound can be thermally decomposed and carbon contained in the magnet particles can be burned off before sintering (i.e., carbon content can be reduced). Therefore, little carbide is formed in a sintering process. Consequently, the entirety of the magnet can be sintered densely without making a gap between a main phase and a grain boundary phase in the sintered magnet and decline of coercive force can be avoided. Further, considerable alpha iron does not separate out in the main phase of the sintered magnet and serious deterioration of magnetic properties can be avoided.

Still further, in the process of calcining the magnet powder or the compact body, the compact body is held for predetermined length of time within a temperature range between 200 and 900 degrees Celsius, more preferably, between 400 and 900 degrees Celsius. Therefore, carbon contained in the magnet particles can be burned off more than required.

As a result, carbon content remaining after sintering is 0.1 wt% or less, or more preferably, 0.05 wt% or less. Thereby, the entirety of the magnet can be sintered densely without occurrence of a gap between a main phase and a grain boundary phase and decline in residual magnetic flux density can be avoided.

In the second manufacturing method, calcination process is performed to the powdery magnet particles, therefore the thermal decomposition of the remaining organic compound can be more easily performed to the entirety of the magnet particles in comparison with a case of calcining compacted magnet particles. That is, it becomes possible to reliably decrease the carbon content of the calcined body. By performing dehydrogenation process after calcination process, activity level is decreased with respect to the calcined body activated by the calcination process. Thereby, the resultant magnet particles are prevented from combining with oxygen and the decrease in the residual magnetic flux density and coercive force can also be prevented.

Not to mention, the present invention is not limited to the above-described embodiment but may be variously improved and modified without departing from the scope of the present invention.

Further, of magnet powder, milling condition, mixing condition, calcination condition, dehydrogenation condition, sintering condition, etc. are not restricted to conditions described in the embodiment.

Incidentally, in the embodiments, a wet bead mill is used as a means for wet-milling the magnet powder; however, other wet-milling methods may be used. For instance, Nanomizer (trade name of a wet-type media-less atomization device manufactured by Nanomizer, Inc.) may be used.

### EXPLANATION OF REFERENCES

- 1: permanent magnet
- 11: main phase
- 12: Nd-rich phase
- 91: main phase
- 92: grain boundary phase
- 93: alpha iron phase

## Claims

1. A manufacturing method of a Nd-Fe-B based permanent magnet, comprising 26.7 to 37 wt% Nd, 60 to 75 wt% Fe, and 1 to 2 wt% B, wherein the method comprises the steps of wet-milling magnet material in an organic solvent to obtain magnet powder;
calcining the magnet powder in hydrogen atmosphere so as to obtain a calcined body; performing a dehydrogenation process to remove hydrogen in the calcined body so that the activity level is depressed with respect to the calcined body activated in the step of calcining, by holding the calcined body in vacuum atmosphere for one through three hours at 200 through 600 degrees Celsius;
compacting the calcined body of which activity level is depressed so as to form a compact body; and
sintering the compact body;
wherein the activity level represent a level of tendency of Nd to combine with oxygen.

2. The manufacturing method of a permanent magnet according to claim 1, wherein residual carbon content after sintering is 0.1 wt% or less.

## Patentansprüche

1. Herstellungsverfahren für einen Nd-Fe-B-basierten Permanentmagneten, umfassend 26,7 bis 37 Gew.-% Nd, 60 bis 75 Gew.-% Fe, und 1 bis 2 Gew.-% B, wobei das Verfahren die Schritte umfasst: Nassmahlen von magnetischem Material in einem organischen Lösungsmittel, um Magnetpulver zu erhalten;
Kalzinieren des Magnetpulvers in Wasserstoffatmosphäre, so dass ein kalzinierter Körper erhalten wird;
Durchführen eines Dehydrierungsprozesses, um Wasserstoff in dem kalzinierten Körper zu entfernen, so dass der Aktivitätsgräd verringert wird in Bezug auf den kalzinierten Körper, der im Schritt des Kalzinierens aktiviert wird, durch Halten des kalzinierten Körpers in Vakuumatmosphäre für 1 bis 3 Stunden bei 200 bis 600° C;
Verdichten des kalzinierten Körpers, dessen Aktivitätsgrad verringert ist, um einen verdichteten Körper zu bilden; und
Sintern des verdichteten Körpers;
wobei der Aktivitätsgrad den Grad der Tendenz von Nd, sich mit Sauerstoff zu verbinden, darstellt.

2. Herstellungsverfahren für einen Permanentmagneten gemäß Anspruch 1, wobei der verbleibende Kohlenstoffanteil nach dem Sintern 0,1 Gew.-% oder weniger ist.

## Revendications

1. Procédé de fabrication d'un aimant permanent à base de Nd-Fe-B, comprenant de 26,7 % en poids à 37 % en poids de Nd, de 60 % en poids à 75 % en poids de Fe, et de 1 % en poids à 2 % en poids de B, dans lequel le procédé comprend les étapes suivantes:
le broyage humide d'un matériau d'aimant dans un solvant organique afin d'obtenir une poudre d'aimant;
la calcination de la poudre d'aimant dans une atmosphère d'hydrogène de manière à obtenir un corps calciné;
l'exécution d'un procédé de déshydrogénation dans le but d'éliminer l'hydrogène dans le corps calciné de telle sorte que le niveau d'activité soit déprimé par rapport au corps calciné activé lors de l'étape de calcination, en maintenant le corps calciné dans une atmosphère sous vide, pendant une à trois heures à 200 à 600 degrés Celsius;
le compactage du corps calciné dont le niveau d'activité est déprimé de manière à former un corps compact; et
le frittage du corps compact,
dans lequel le niveau d'activité représente un niveau de tendance du Nd à se combiner avec l'oxygène.

2. Procédé de fabrication d'un aimant permanent selon la revendication 1, dans lequel la teneur en carbone résiduel après le frittage est de 0,1 % en poids, ou moins.
